

Nov. 10, 1931.

C. WINKLER

1,831,761

METHOD OF PRODUCING PACKING FOR THE IMPRESSION  
CYLINDER OF PRINTING MACHINES  
Filed May 27, 1930

Fig. 1



Fig. 2



INVENTOR

Carl Winkler  
BY *Miner & Co.*

ATTORNEYS

## UNITED STATES PATENT OFFICE

CARL WINKLER, OF BERN, SWITZERLAND

## METHOD OF PRODUCING PACKING FOR THE IMPRESSION CYLINDER OF PRINTING MACHINES

Application filed May 27, 1930, Serial No. 456,086, and in Germany September 22, 1928.

My invention relates to a method of producing a packing suitable for the impression cylinder of printing machines, and the new feature consists in adding to a paper or cardboard pulp—hereinafter called paper pulp—  
5 some elastic stuff, preferably cork, in finely divided condition.

In carrying out my invention the cork, or other elastic material, is mixed well with the paper pulp, by mechanical, or hand, stirring,  
10 and, in the paper or cardboard making machine, the mixture is made up into one or more layers. This can be done in the usual way by a sieve cylinder which dips into the mixture of paper pulp and cork, or the like, and applies a thin layer to a felt, which contacts with another cylinder, on which the pulp is applied in several layers over each other.

With the object of still further increasing  
20 the elasticity of the packing, rubber, in the form of latex, can be added to the paper pulp.

By experiment it has been found that cork can be mixed with paper pulp if the cork is sufficiently finely divided, and care is taken  
25 to prevent the cork from collecting in irregular bunches near the sieve cylinder.

In the drawings a machine for making the packing according to my invention is shown by way of example,

30 Fig. 1 being a diagrammatic side elevation, and

Fig. 2 a plan.

The perforated or sieve cylinder *a* rotates, as usual in a vat *b* and transfers a layer of  
35 paper pulp to the felt belt *c* which runs over the rolls *d*, *e* and transfers one layer after the other to the cylinder *f*. On this cylinder *f* the sheets formed by the repeated layers of strained pulp applied are periodically cut  
40 longitudinally and removed from the cylinder.

In the vat *b* cork, in very finely divided condition, is added to the pulp and well mixed with same by stirring. During the stirring  
45 process, rubber in the condition known as "latex" can be added.

What I desire to secure by Letters Patent is:

50 The method of producing packing for the impression cylinders of printing machines

which consists in mixing paper pulp with cork powder and rubber in the form of latex, and forming a sheet from said mixture.

In testimony whereof I have signed my name to this specification.

CARL WINKLER.

55

60

65

70

75

80

85

90

95

100